

Feb. 3, 1959

M. WEINBERG ET AL

2,871,550

COMPOSITE CHROMIUM ELECTROPLATE AND METHOD OF MAKING SAME

Filed Jan. 10, 1958



1

2,871,550

COMPOSITE CHROMIUM ELECTROPLATE AND  
METHOD OF MAKING SAME

Max Weinberg, Detroit, and Henry Brown, Huntington Woods, Mich., assignors to The Udylite Research Corporation, Detroit, Mich., a corporation of Michigan

Application January 10, 1958, Serial No. 708,267

18 Claims. (Cl. 29—183.5)

This invention relates to a bright chromium finished electroplate having improved corrosion resistance, and to the method for producing the same.

Conventional bright "chrome" plate intended to withstand outdoor exposure, consists usually of nickel electroplate of 1 to 2 mils thickness with a final thin (0.01—0.02 mil) deposit of bright chromium electroplate, or it consists of copper-nickel-chromium electroplate of about 0.5 to 1 mil of copper, and 1 to 1.5 mils of nickel and a final thin bright chromium plate of about 0.01 to 0.02 mil thickness. It is well-known that the corrosion protection of such composite coatings is primarily attributable to the nickel layer, and the degree of protection is dependent mainly on the thickness of the nickel layer. Furthermore, it is now well-known that the thin final layer of the bright non-tarnishing chromium plate actually decreases the corrosion protection value of bright nickel plate underneath it, and the outdoor exposure results with such chrome plate in an industrial or marine atmosphere leaves much to be desired. This invention is based on the discovery of a composite chromium-nickel-chromium electroplated coating having certain critical thickness relationships between the successive layers thereof which provide an unexpectedly superior corrosion-resistance while employing substantially less nickel than normally used for outdoor corrosion protection.

In accordance with this invention, it has now been found that by using a thickness of chromium plate of 0.03 to about 0.2 mil thick underneath 0.2 to 2 mils thick nickel plate followed by a final bright chromium plate of 0.005 to 0.1 mil thickness, it is possible to obtain extraordinary corrosion protection in outdoor exposure for industrial metals susceptible to atmospheric corrosion such as steel, iron, aluminum and its alloys, magnesium and its alloys, copper, zinc and its alloys, brasses, etc.

For example, it has now been found that by using about 0.1 to 0.15 mil of chromium plate underneath about 0.5 to 1 mil of nickel plate followed by a final bright chromium plate of 0.03 to 0.06 mil thickness, it is possible to obtain outstanding corrosion protection in outdoor exposure compared to 2 mils nickel plate with the usual thin chromium plate. With thinner composite coatings of this invention, for example, the composite coating consisting of 0.03 mil chromium underneath 0.2 mil of nickel followed by thin (0.005 to 0.02 mil) final chromium plate, the corrosion protection obtained is superior to copper-nickel or nickel plate of 0.5 to 0.7 mil thickness with the same final chromium plate exposed in an outdoor industrial atmosphere. Using only 0.2 mil nickel with 0.1 to 0.2 mil of chromium plate underneath and 0.03 mil of final chromium plate, the outdoor exposure results obtained were outstanding compared to 1 mil thick nickel plate with the usual 0.01 mil of final chromium plate. On the basis of many tests it was found that the first chromium plate should be at least 0.03 mil thick and that the minimum thickness for the nickel plate overlying

2

this chromium plate should be 0.2 mil, whereas the final bright chromium plate could vary from 0.005 to 0.1 mil thickness and still have consistently excellent outdoor corrosion results. There is no need for thicknesses of nickel greater than 2 mils sandwiched between the chromium plates, to obtain outstanding outdoor corrosion protection, in even the most severe conditions of outdoor exposure in an industrial atmosphere. In fact, as already mentioned, 1 mil thickness of nickel sandwiched between 0.1 mil of underlying chromium and 0.03 mil of final chromium is superior to 2 mils of nickel with the usual final thin chromium plate. The use of more than 0.2 mil of chromium underneath the nickel is not necessary, and does not add any substantial improvement in outdoor corrosion protection in the composite coatings of this invention. Thus, this invention encompasses the use of a composite electroplate consisting of, chromium plate of 0.03 to about 0.2 mil thick underneath a nickel plate of 0.2 to about 2 mils thick followed by a final chromium plate of 0.005 to about 0.1 mil thickness to give extraordinary outdoor corrosion protection to such metals as steel, aluminum and its alloys, zinc and its alloys, magnesium and its alloys, copper and brasses.

The following outdoor exposure results obtained in an industrial atmosphere of a northern mid-western city of the United States in an area heavily contaminated with the smoke from trains, illustrate the magnitude of the improvement in corrosion protection obtained with the use of the composite coating of this invention.

In a series of 6" x 4" steel panels plated with about 0.1 mil of chromium plate deposited from a 130° F.—150° F. warm chromium plating bath (32—40 oz./gal. CrO<sub>3</sub>, and a ratio of CrO<sub>3</sub> to SO<sub>4</sub> of about 125 to 1 to about 200 to 1) followed by a nickel plate of only 0.5 mil thickness, and a bright final chromium plate of 0.01 to 0.03 mil thick, the outdoor corrosion protection afforded the steel was far superior to coatings consisting of twice the thickness of nickel plate with the same final chromium plate. When the latter conventional coatings had already shown from 100 to 500 rust spots per square foot, the former still had no rust spots on most of the panels, with only an occasional 1 or 2 rust spots on some of the panels. Furthermore, the underside (where dew condensation is most pronounced) of these outdoor exposed panels (exposed at 45° angle) were also free from corrosion whereas the conventional panels without the approximately 0.1 mil chromium underneath the nickel plate were very rusty at the end of one year outdoor exposure.

Excellent results with the above described composite coating of chromium-nickel-chromium were also obtained in such accelerated tests as salt-spray, acetic acid modified salt-spray (salt-spray with 5% salt solution containing acetic acid to give a pH of 3.2), and Corrodkote. Corrodkote is an accelerated corrosion test employing a corrosive coating applied to the chrome plated surface, the coating consisting of kaolin mixed with a solution of ammonium chloride, ferric chloride and cupric nitrate, and then this coated surface is submitted to 90% humidity for 20 hours. This test procedure is described more completely in Proceedings of the American Electroplaters Society, vol. 43, pp. 50—55 (1956). When the Corrodkote test was used with 100% humidity instead of 90% humidity conditions, the above described chromium-nickel-chromium coating gave excellent results, whereas, conventional coatings of 1.5 mil thickness of nickel or copper-nickel covered with the same final thickness of bright chromium gave very poor results.

The results in outdoor exposure in an industrial atmosphere of a northern mid-western city of the United States,

in an area heavily contaminated with the smoke from trains, especially during the late fall, winter and early spring months when corrosion failure of "chrome" plate (the usual copper-nickel-chromium plate or nickel-chromium plate) is the most severe, indicated that with the composite plate of this invention the corrosion pits starting from pores in the final chromium plate and penetrating through the nickel plate were greatly retarded or practically stopped on reaching the underlying chromium plate of at least 0.03 mil thickness. If the underlying chromium plate was below about 0.02 mil thickness, usually erratic results were obtained, in that most often no dramatic enhancement of corrosion protection resulted from the presence of such a thin chromium plate underneath the nickel plate, or at least the enhancement was not significant enough to be worth the extra steps of applying the thin (0.01-0.02 mil) intermediate chromium plate. Apparently when the underlying chromium plate is only about 0.01 to 0.02 mil thick, it is most often penetrated too quickly before the exposed chromium can recover its passivity. The surface of the underlying chromium plate had been necessarily rendered active by plating it in a low pH nickel strike before the regular nickel plate of 0.2 mil or thicker was applied. Thus, if the chromium plate exposed underneath the corrosion pit in the nickel is of such a thickness (at least about 0.03 mil) that it can become passive before it is penetrated, the corrosion cell set up by the presence of a film or layer of weakly acidic or saline electrolyte on top of the porous final thin chromium plate will tend to develop a corrosion pit which tends to move laterally in the nickel instead of downward, thus greatly superior protection of the metal underneath the lower layer of chromium is accomplished without any blistering effects or unsightly corrosion products because of the very slow corrosion attack of nickel compared, for example, to copper or zinc, or iron. This appears to be the explanation of the dramatic improvement in corrosion protection obtained when the chromium is at least 0.03 mil thick underneath at least 0.2 mil of nickel plate.

Figures 1-5 are illustrative diagrams of the corrosion cell involved in outdoor exposure of nickel-chromium plate in an industrial or marine atmosphere. In Figures 1 and 5 are shown the diagrams of the corrosion cell involved when the composite chromium-nickel-chromium plate of this invention is on steel exposed in a damp industrial or marine atmosphere. Figure 2 illustrates the case when no chromium plate is underneath the nickel plate. Figure 3 illustrates the case when the underlying chromium plate is very thin, i. e., less than about 0.2 mil. Fig. 4 shows a thick nickel plate on the basis metal with a conventional chromium overlayer. In each of the figures a corrosion pit is shown which started at a pore designated  $\alpha$  in the final thin chromium plate A. The corrosion pit is the type that results when this chromium plate is covered with a layer of weakly acidic or saline electrolyte, which sets up a galvanic corrosion cell, with a passive final chromium plate as cathode, indicated by negative electrical signs in the diagrams, and the metal (nickel) exposed in the pore of the final thin chromium as anode, indicated by positive electrical signs. If the nickel plate is thin, e. g. 0.2 to 0.5 mil, then it will not take long before the nickel plate is penetrated and the more readily corrodible iron is attacked when there is no underlying chromium plate, or very thin chromium plate, as may be seen in Figures 2 and 3, respectively. With thicker nickel plate (1.5 to 2 mil), it will take much longer for the corrosion pit to reach the iron or steel, as illustrated in Fig. 4. However, with a chromium plate of about 0.03 to 0.2 mil underlying the nickel plate, as shown in Fig. 1, the corrosion pit tends to go laterally in the nickel plate on reaching the underlying chromium plate instead of downward, thus protecting the more readily corrodible base metal (Fe, Al, Zn, Mg, Cu, brass, etc.) underneath, in a much more effective manner.

than with much thicker nickel plate carrying the same final chromium plate, but having no chromium plate of a thickness of about 0.03 mil to 0.2 mil underneath the nickel plate. Figure 5 illustrates the case when the final thin chromium plate is of the usual 0.005 to 0.02 mil thickness and shows the appearance of the corrosion pit after 1 year of exposure to an industrial atmosphere. Figure 1 shows the typical appearance after 1 year exposure in an industrial atmosphere when the thickness of the final chromium plate is in the range of 0.03-0.05 mil, and was plated from a 120° F.-140° F. hexavalent chromium bath.

The outdoor corrosion protection afforded to steel, iron, aluminum, zinc, etc. by the composite coating of, for example, 0.06 to 0.2 mil of chromium from a 120°-180° F. warm hexavalent chromium plating bath underneath 0.5 to 1 mil of bright nickel followed by 0.03 mil of final bright chromium from a 130° F. hexavalent chromium bath, is superior to the same nickel plate with a total final chromium plate equal to the underlying and overlying chromium plate thickness. Furthermore, such thick final chromium coatings must be polished to be bright and are very impractical to use for bright, high lustre coatings because of the excessive costs to polish them to a high lustre, whereas, by using a semi-bright or dull chromium plate of about 0.08 to 0.2 mil thickness preferably from warm (120° F.-180° F.) hexavalent chromium plating baths, it is possible to cover this plate with a bright deposited nickel plate that will brighten up the dull or semi-bright chromium to full bright lustre for the final thin bright chromium plate. Thus, by distributing the thicker values (0.1 to 0.2 mil) of the chromium plate underneath and on top of a nickel plate, it is not only possible to obtain a minimum of stress-cracking of the final bright chromium plate, but also to avoid polishing a thick semi-bright or dull chromium plate of minimum stress-cracks, and there is also obtained dramatically superior outdoor corrosion protection which is far superior to bright nickel plate of double the total thickness with the same final thin bright chromium plate. The main reason for this lies in the favored lateral corrosion of the nickel plate sandwiched between the chromium plate of 0.03 to 0.2 mil thickness and the final thin bright chromium deposit, as already explained, and diagrammatically illustrated in Figures 1 and 5.

This sequence of chromium plate of 0.03 to 0.2 mil followed by 0.2 to 2 mils of nickel followed by a final chromium plate of 0.005 to 0.1 mil thickness, used directly on zinc, or its alloys, aluminum or its alloys, or on magnesium, or on copper or brass provides the same excellent protection in outdoor exposure that is given to steel. The aluminum can often be plated directly, or it can first be anodized or partially anodized before plating, or covered with a zinc film (as from an immersion zincate solution or fluoborate solution), or covered with an immersion zinc film or zinc electroplate, and a copper plate or brass plate, before applying the above described chromium-nickel-chromium plate. The composite chromium-nickel-chromium plate of this invention applied to aluminum or aluminum alloys as already described gives far more superior corrosion protection than the usual heavy copper-nickel-chromium coatings of at least a total of 2 to 3 mils thickness applied to aluminum, and can be used on high strength aluminum alloys that do not yield a bright anodized finish. In this way aluminum and its alloys can be given the high lustre of "chrome" plate but with excellent outdoor corrosion resistance instead of the usual corrosion blistering resulting from the present conventional copper-nickel-chromium coatings. Zinc metal or zinc alloys such as zinc base die-cast can satisfactorily first be copper plated or brass plated or nickel plated before starting the sequence of the above described composite chromium-nickel-chromium plate.

The preferred chromium plate for use underneath the nickel plate is that obtained from warm hexavalent chromium baths operated at about 120° F. to 180° F., which

yield chromium plate with minimum stress. The underlying chromium plate may be dull, semi-bright or bright, though it is preferred to be semi-bright or even dull, and actually excellent results are also obtained with lower temperature 60° F.-70° F. (even refrigerated to 50° F.) chromium plating baths, especially with such baths as the chromium plating bath described in French Patent 754,299, which can be used to plate zinc die-cast directly. Alternatively the underlying chromium plate may be deposited by a contact process such as by brush plating, as in the "Dalic" process as described in Electroplating, vol. 6, No. 4, p. 131 (1953). The presence of an overlying nickel plate of at least 0.2 mil thickness tends to make the differences between various chromium plates (as obtained from warm versus cold baths) less important than when compared without the overlying nickel plate. Nevertheless, the underlying chromium plate should be of minimum stress for best results.

In depositing the thicker underlying chromium plate on complex shaped articles (articles with deep recesses), it is best to use conforming or auxiliary anodes to obtain optimum distribution of the first chromium plate. Then after rinsing thoroughly, the parts can be re-racked without using conforming anodes for the subsequent nickel and final chromium plate. On simpler shaped articles the use of conforming or auxiliary anodes for the first chromium plate are of course not needed. In any case, after the first chromium plate of at least 0.03 mil to about 0.2 mil is deposited, the articles are thoroughly rinsed including a dip or preferably an agitated soak in a water solution of a reducing agent capable of reducing hexavalent chromium to trivalent chromium, such as compounds containing sulfur with a valence less than +6 in anion form including sodium bisulfite, sodium sulfite, hydro-sulfite and thiosulfate. Other reducing agents such as aqueous solutions of hydrogen peroxide, sugars or ferrous salts can be used to reduce the last traces of chromic acid on the work or rack that might not have been rinsed off. In addition sequestering agents capable of preventing the precipitation of Cr(OH)<sub>3</sub> in the reducing solutions is advantageously incorporated such as sodium gluconate, nitrilotriacetate, ethylene diamine tetra-acetates, etc. After further rinsing, the chromium plated articles are given a low pH nickel strike for example, from nickel strike baths such as the following: 24 oz./gal. NiCl<sub>2</sub>.6H<sub>2</sub>O with 5% to 10% by volume of hydrochloric acid; or 12 oz./gal. NiSO<sub>4</sub>.6H<sub>2</sub>O+12 oz./gal. NiCl<sub>2</sub>.6H<sub>2</sub>O and 5% to 10% by volume of hydrochloric acid, with or without boric acid present; or from nickel sulfate baths containing 10% to 20% sulfuric acid. After about a 1 to 10 minute nickel strike plate is made at cathode current densities of 10-100 amps./sq. ft., the articles are transferred with or without rinsing to regular nickel plating baths of the Watts type, high chloride type, fluoborate or sulfamate type, etc. These nickel baths can be used with addition agents to give semi-bright or bright nickel plating or a series of nickel baths can be used combining dull nickel, semi-bright nickel with final bright nickel. It is preferred to use bright nickel or a combination of a semi-bright nickel and bright nickel. After obtaining a bright surface either by buffering the semi-bright or by bright nickel plating, the nickel surface is given the usual final thin bright chromium plate. It is preferred to use a final bright chromium plate from a 120° F.-140° F. bath (preferably about 130° F.) for a thickness of 0.03 to about 0.08 mil. In general, however, the thickness for the final chromium plate need not be greater than about 0.03 mil for very excellent results, and can be the usual bright chromium plate from the room temperature to 140° F. baths.

The preferred underlying chromium plate of 0.03 to 0.2 mil thickness of semi-bright or dull chromium of minimum stress and of maximum corrosion resistance, is best brightened, as already suggested, by the use of semi-bright high-leveling nickel plating followed by fully bright nickel, or by fully bright nickel alone, and this way la-

borious and expensive buffing of a thick semi-bright or dull chromium surface is avoided. Not only is it expensive to buff or polish thick chromium plate, as already mentioned, but it also causes a significant loss in corrosion resistance of the chromium plate itself. Whereas, by covering the unpolished underlying chromium plate with a nickel coating of equal or greater thickness than the chromium plate, the effect of any residual stresses in the underlying chromium plate is decreased by being sandwiched between more ductile metal.

The above described sequence of chromium plate followed by nickel followed by chromium can be used on stainless steel with beneficial effects. While stainless steel, especially chromium plated stainless steel gives superb results in outdoor exposure, it nevertheless is difficult to obtain a high lustre on stainless steel by polishing because of its "work-hardening" qualities. If stainless steel is given a nickel strike and then brightened by application of bright nickel plate, it loses its great resistance to rusting because the use of the low pH nickel strike results in removal of the passive film of the stainless steel. Whereas, if the stainless steel is plated with the sequence of chromium-nickel-chromium as given above, that is, chromium plated first from the hexavalent chromium bath with a thickness of about 0.03 mil chromium and then given a low pH nickel strike and bright nickel plated with about 0.2 to 0.5 mil nickel, and given a final thin (0.01-0.03 mil) bright chromium plate, it is possible to brighten up the stainless steel with bright nickel to a high lustre without a serious loss of corrosion resistance. The term "stainless steel" is intended in its conventionally understood sense.

In the case of brass articles, it is not as important, because of the excellent corrosion resistance of nickel-chromium plated brass, to use the above described sequence of chromium-nickel-chromium plate, as it is for steel, aluminum, magnesium, and zinc, nevertheless, it makes possible even superior outdoor corrosion protection with thinner nickel plate than is usually used. Thus, instead of 0.5 to 0.8 mil nickel plate, only about 0.2 mil nickel plate sandwiched between coatings of 0.03 mil of chromium is all that is needed.

In general, before the application of the sequence of the above described composite chromium-nickel-chromium plate, electroplates of copper, brass, zinc, or nickel could be used on the basis metal. In each case, outstanding corrosion protection is conferred to the underlying metal by the above described composite chromium-nickel-chromium electroplate sequence.

The following examples further illustrate the use of the composite chromium-nickel-chromium electroplate of this invention to obtain bright "chrome" finished articles of outstanding corrosion resistance to outdoor exposure.

#### EXAMPLE I

##### *Steel basis metal*

Polished steel suitable for use as automobile bumpers is cleaned in the conventional manner and after a final alkaline anodic cleaner, rinsed, acid dipped or anodically etched, and then given a chromium plate of 0.1 to 0.2 mil thickness from the following hexavalent chromium bath:

|                               |                                |
|-------------------------------|--------------------------------|
| CrO <sub>3</sub> -----        | 40 oz./gal. (325 grams/liter). |
| SO <sub>4</sub> -----         | 4 oz./gal. (3.25 grams/liter). |
| Temperature -----             | 140° F.-160° F.                |
| Cathode current density ----- | 400-500 amps./sq. ft.          |

Plating time ----- 10-20 minutes.

After the initial chromium plating is finished, the bumpers are thoroughly rinsed, and given an agitated soak dip in a 5% solution of sodium sulfite, rinsed thoroughly in

water and transferred to a low pH nickel strike such as the following:

|                                                                                                   |         |    |
|---------------------------------------------------------------------------------------------------|---------|----|
| NiSO <sub>4</sub> .6H <sub>2</sub> O                                                              | oz./gal | 12 |
| NiCl <sub>2</sub> .6H <sub>2</sub> O (or lower nickel chloride and higher nickel sulfate content) | oz./gal | 12 |
| H <sub>3</sub> BO <sub>3</sub>                                                                    | oz./gal | 4  |
| 5%-10% by volume of concentrated hydrochloric acid                                                |         |    |

Room temperature

|                         |               |       |
|-------------------------|---------------|-------|
| Cathode current density | amps./sq. ft. | 20-30 |
| Plating time            | minutes       | 3-5   |

After removal from the nickel strike, the bumpers are then transferred to a ductile semi-bright type Waits nickel plating bath containing an addition agent selected from the class consisting, for example, of bromal, chloral hydrate and 8-methoxy coumarin, and plated with about 0.8 mil to 1 mil of semi-bright nickel and transferred to a bright nickel plating bath containing a brightener selected from the class consisting of benzene sulfonamides and sulfonimides especially o-benzoyl sulfimide, together with an aliphatic unsaturated compound or compounds, and plated with about 0.2 to 0.3 mil of bright nickel, then rinsed and transferred to a chromium bath of approximately the following composition:

|                         |               |         |
|-------------------------|---------------|---------|
| CrO <sub>3</sub>        | oz./gal       | 33      |
| SO <sub>4</sub>         | oz./gal       | 1.5-2   |
| Temperature             | °F            | 131     |
| Cathode current density | amps./sq. ft. | 285-325 |

and plating a thickness of bright chromium of 0.03 to 0.05 mil.

#### EXAMPLE II

##### Steel basis metal

Polished steel bumper guards are put through the same steps given in Example I except that the first chromium plating bath is operated at 130° F. and about 300 amps./sq. ft. and a chromium plate of about 0.1 mil is applied, and after the nickel strike is applied, the articles are transferred directly to the bright nickel bath and given about a 1 mil thick nickel plate, and then a final chromium plate of 0.03 to 0.06 mil thickness from a 120° F.-140° F. hexavalent chromium bath.

#### EXAMPLE III

##### Aluminum basis metal

After employing the usual methods of cleaning aluminum and its alloys, the clean aluminum is given a dip in an alkaline zincate solution for 10 seconds to about 60 seconds, then rinsed and given a copper strike from a low metal low free cyanide copper bath and using low cathode current densities (about 5 to 10 amps./sq. ft.), and the copper plating continued until about 0.1-0.3 mil of copper is deposited and then after rinsing, the chromium-nickel-chromium electroplate sequence is applied as given in Example II above.

#### EXAMPLE IV

##### Zinc base die-cast metal

After employing the usual methods of cleaning zinc die-cast metal, the zinc die cast is plated with smooth copper plate from a cyanide copper or pyrophosphate copper bath to a thickness of 0.3 to 0.4 mil of copper and then after rinsing, the chromium-nickel-chromium electroplate is applied as given in Example II above. Instead of the copper plate directly on the zinc, a Bornhauser chromium plate can be applied directly on the zinc to a thickness of 0.2 mil, then the nickel and final bright chromium applied as described in Example II above. The Bornhauser chromium plating bath is as follows:

|                  |         |     |
|------------------|---------|-----|
| CrO <sub>3</sub> | oz./gal | 53  |
| NaOH             | oz./gal | 7.7 |

|                                |               |         |
|--------------------------------|---------------|---------|
| Cr <sub>2</sub> O <sub>3</sub> | oz./gal       | 1.0     |
| H <sub>2</sub> SO <sub>4</sub> | oz./gal       | 0.1     |
| Temperature                    | °F            | 60-70   |
| Current density                | amps./sq. ft. | 200-800 |

5 Articles plated in accordance with this example are suitable for use outdoors or as laboratory hardware, such as faucet handles, etc.

#### EXAMPLE V

##### Magnesium and magnesium-alloy basis metals

After the usual methods of cleaning and preparation of the surface of the magnesium articles is completed, for example, according to directions given in Bulletin No. DM108b of the Magnesium Department of the Dow Chemical Co., Midland, Michigan, and the magnesium has been given a zinc immersion coating and a copper plate of about 0.1 to 0.3 mil thick, it is then given the chromium-nickel-chromium electroplate sequence as described in Example II above.

10 The plated surfaces resulting from the process above specified in Examples I and II were subjected to outdoor corrosion in the northern mid-west section of the United States, and upon inspection at the end of one year showed no evidence of corrosion. Test panels of the same type metal given a conventional copper-nickel-chromium coating with the nickel thickness being similar to that specified in Examples I and II when subjected to the same outdoor corrosion showed from 100-500 rust spots per square foot.

15 The aluminum, zinc and magnesium plated in accordance with the procedures set forth in Examples III, IV and V respectively, when subjected to the Corrodokote test, which simulates one year of outdoor exposure, show no evidence of blistering. For the best corrosion protection of steel articles that will undergo deformation in service, as for example, automobile bumpers and bumper-guards, etc., it was found that by using an underlying plate of zinc or cadmium or alloys thereof which are anodic to steel of about 0.1 to 0.5 mil thickness beneath the chromium-nickel-chromium plate, that no rusting occurred with severe distortion of the plated steel articles on outdoor exposure for extended periods of time. The zinc, cadmium, or anodic-to-steel alloy thereof can be coated directly with the chromium-nickel-chromium plate of this invention, or a 0.1-0.3 mil coating of copper or yellow brass can be, and sometimes is preferably, plated directly on the zinc, cadmium or anodic-to-steel alloy coating prior to the plating of the chromium-nickel-chromium plate. In this aspect of the invention the electroplate which underlies the chromium-nickel-chromium coating of this invention may be a single or a composite coating which is at least in part anodic-to-steel, for example a zinc coating directly on the steel surface which is overlaid with an adherent copper coating. However, even without this additional anodic-to-steel plate underneath the lower thick chromium plate, it is surprising how little rusting occurs with severely distorted chromium-nickel-chromium plated steel articles.

#### EXAMPLE VI

20 Steel of the type used in Example I, after cleaning is given a zinc plate of 0.2 to 0.5 mil thickness, from a zinc cyanide bath, and then a copper strike of 0.1-0.2 mil thickness from a cyanide copper bath. This surface is then chromium-nickel-chromium plated as in Example I.

25 This produces a composite plated surface that even when severely distorted, has excellent corrosion resistance.

What is claimed is:

30 1. A laminated corrosion-protective final coating on a metal base susceptible to atmospheric corrosion comprising a layer of chromium having a thickness in the range of about 0.03 to about 0.2 mil, nickel overlying said chromium and adherent thereto and having a thickness in the range of about 0.2 mil to about 2 mils, and chromium overlying said nickel and adherent thereto and having a

thickness in the range of about 0.005 mil to about 0.1 mil.

2. A laminated corrosion-protective final electroplate on a metal base susceptible to atmospheric corrosion comprising a layer of adherent electroplated chromium having a thickness in the range of about .06 to about .15 mil, electroplated nickel overlying said chromium and adherent thereto and having a thickness in the range of about 0.5 to 1 mil, and electroplated chromium overlying said nickel and adherent thereto and having a thickness in the range of about 0.03 mil to about 0.08 mil.

3. A laminated corrosion-protective final electroplate on a metal base of the class consisting of iron, steel, stainless steel, copper, brass, aluminum and its alloys, magnesium and its alloys and zinc and its alloys consisting of electroplated chromium having a thickness in the range of about 0.03 to about 0.2 mil, electroplated nickel overlying said chromium and adherent thereto and having a thickness in the range of about 0.2 mil to about 2 mils, and electroplated chromium overlying said nickel and adherent thereto and having a thickness in the range of about 0.005 mil to about 0.1 mil.

4. A coating in accordance with claim 1 wherein said nickel plate comprises a semi-bright portion overlaid by a bright portion.

5. A coating in accordance with claim 1 wherein said nickel plate is substantially all bright nickel.

6. A composite corrosion-protective electroplated final coating on steel consisting of a first electroplate, at least a part of which is anodic-to-steel and is an electroplated metal selected from the group consisting of zinc, cadmium and the anodic-to-steel alloys thereof, adherent electroplated chromium overlying said first electroplate and having a thickness in the range of about 0.03 to 0.2 mil, electroplated nickel overlying said chromium and adherent thereto and having a thickness in the range of about 0.2 mil to about 2 mils, and electroplated chromium overlying said nickel and adherent thereto and having a thickness in the range of about 0.005 mil to about 0.1 mil.

7. A coating in accordance with claim 1 wherein said metal base is steel.

8. A coating in accordance with claim 3 wherein said metal base is aluminum and its alloys.

9. A coating in accordance with claim 3 wherein said metal base is zinc and its alloys.

10. A coating in accordance with claim 3 wherein said metal base is magnesium and its alloys.

11. A method for electroplating from aqueous solutions a corrosion-protective composite coating on a metallic surface susceptible to atmospheric corrosion which comprises the steps of electroplating on said surface adherent chromium having a thickness in the range of about 0.03 mil to about 0.2 mil, electroplating on said chromium adherent nickel having a thickness in the range of about 0.2 mil to about 2 mils, and thereafter electroplating on said nickel adherent chromium having a thickness in the range of about 0.005 to 0.1 mil.

12. A method for electroplating from aqueous solutions a corrosion-protective composite coating on a metallic surface susceptible to atmospheric corrosion which comprises the steps of electroplating on said surface adherent chromium having a thickness in the range of about .06 to about 0.15 mil, electroplating on said chromium adherent nickel having a thickness in the range of about 0.5 to 1 mil, and thereafter electroplating on said nickel adherent chromium having a thickness in the range of about 0.03 mil to about .08 mil.

13. A method for electroplating from aqueous solutions a corrosion-protective composite coating on a metal base of the class consisting of iron, steel, stainless steel, copper, brass, aluminum and its alloys, magnesium and its alloys and zinc and its alloys which comprises the steps of electroplating on said surface adherent chromium having a thickness in the range of about 0.03 mil to about 0.2 mil, electroplating on said chromium adherent nickel

having a thickness in the range of about 0.2 mil to about 2 mils, and thereafter electroplating on said nickel adherent chromium having a thickness in the range of about 0.005 to about 0.1 mil.

14. A method for electroplating from aqueous solutions a corrosion-protective composite coating on a metal base of the class consisting of iron, steel, stainless steel, copper, brass, aluminum and its alloys, magnesium and its alloys and zinc and its alloys which comprises the steps of electroplating on said surface adherent chromium having a thickness in the range of about .06 to about .15 mil, electroplating on said chromium adherent nickel having a thickness in the range of about 0.5 to 1 mil, and thereafter electroplating on said nickel adherent chromium having a thickness in the range of about .03 mil to about .08 mil.

15. A method for electroplating from aqueous solutions a corrosion protective composite coating on a metallic surface susceptible to atmospheric corrosion which comprises the steps of electroplating on said surface an adherent chromium plate having a thickness in the range of about 0.03 mil to about 0.2 mil, rinsing said chromium-coated surface in an aqueous rinse solution containing a reducing agent capable of reducing the hexavalent chromium ion to the trivalent chromium ion, electroplating on said rinsed chromium coating an adherent nickel plate having a thickness in the range of about 0.2 mil to about 2 mils, and thereafter electroplating on said nickel plate an adherent chromium plate having a thickness in the range of about 0.005 to about 0.1 mil.

16. A method in accordance with claim 15 wherein said aqueous rinse solution contains in addition to said reducing agent a sequestering agent capable of preventing precipitation of chromic hydroxide.

17. A method for electroplating from aqueous solutions a corrosion protective composite coating on a metallic surface susceptible to atmospheric corrosion which comprises the steps of electroplating on said surface a first electroplate, at least a part of which is anodic-to-steel and is an electroplated metal selected from the group consisting of zinc, cadmium and the anodic-to-steel alloys thereof, electroplating on said first electroplate adherent chromium having a thickness in a range of about 0.03 to about 0.2 mil, electroplating on said chromium adherent nickel having a thickness in the range of about 0.2 to about 2 mils, and thereafter electroplating on said nickel adherent chromium having a thickness in the range of about 0.005 to about 0.1 mil.

18. A method for electroplating from aqueous solutions a corrosion protective composite coating on a metallic surface susceptible to atmospheric corrosion which comprises the steps of electroplating on said surface a first electroplate, at least a part of which is anodic-to-steel and is an electroplated metal selected from the group consisting of zinc, cadmium and the anodic-to-steel alloys thereof, electroplating on said first electroplate adherent chromium having a thickness in a range of about 0.06 to about 0.15 mil, electroplating on said chromium adherent nickel having a thickness in the range of about 0.5 to about 1 mil, and thereafter electroplating on said nickel adherent chromium having a thickness in the range of about 0.03 to about 0.08 mil.

65 References Cited in the file of this patent  
UNITED STATES PATENTS  
1,615,585 Humphries ----- Jan. 25, 1927  
2,093,428 Ford et al. ----- Sept. 21, 1937  
70 2,147,407 Huston et al. ----- Feb. 14, 1939  
2,188,399 Bieber ----- Jan. 30, 1940  
2,336,568 Pray ----- Dec. 14, 1943

75 FOREIGN PATENTS  
684,434 Great Britain ----- Dec. 17, 1952